

## UNITED STATES PATENT OFFICE.

ERNEST P. MARS, OF CHICAGO, ILLINOIS.

## FINISHING GRINDING STONE.

No Drawing.

Application filed March 18, 1927. Serial No. 176,581.

My invention relates to artificial stones for abrasive and polishing purposes. Viewed in its general objects, my invention aims to provide a composition stone for this purpose which can easily be manufactured with a highly uniform distribution of the abrasive ingredient, or of both abrasive and polishing ingredients; which will require no poisonous ingredients for its manufacture; and in which the relative proportion and hardness of the abrasive and polishing ingredients can readily be varied according to the material on which the stone is to be used.

15 My invention also provides a composition for this purpose in which the body material (namely the material that has the abrasive and polishing ingredients distributed through it) can be varied considerably in its own hardness; and in which this body material will gradually wear away to form a suitable "muck" when the stone is used for wet grinding, so that this muck can carry off the abraded particles of the material 25 which is being ground; and in which this body material is somewhat abrasive and is of such a nature that the detached particles of the object on which the stone is used will not adhere to this material.

30 In its immediate commercial aspects, my invention is particularly suited for the manufacture of stones to be used in the last step of the grinding of the copper printing cylinders employed on multicolor printing presses, such as the so called "rotogravure" presses. Hence I am describing my invention more particularly with the ingredients proportioned for that purpose, although I do not wish to be limited to these particular proportions or to the abrasive and polishing ingredients hereafter specifically mentioned.

Owing to the high cost of such a copper printing cylinder, it is customary to use the cylinder repeatedly for different imprints 45 by grinding off the raised printing surface and again etching a new surface on it. For this purpose, the raised portions are first ground off by comparatively rough abrasive means, after which the cylinder is subjected to a finish-grinding. To insure a uniform diameter and a freedom from scratches, it is important that the abrasive ingredients in the stone employed for this finish-grinding should be distributed through the stone 50 with a high degree of uniformity, that the body material be uniform in hardness so as not to wear irregularly, that the stone be free from hard spots and unduly hard abrasive portions which would produce scratches, and also that the detached particles of copper 60 will not attach themselves to the stone. No natural stone has yet been found to meet these severe requirements, and even the grinding stones imported for this purpose require a good deal of subsequent hand labor 65 for removing scratches. Moreover, the natural abrasive stones do not afford a sufficient polishing for the cylinders, so that considerable later hand labor is also needed to finish this polishing.

70 In experimenting with various possible body materials for carrying the needed abrasive and polishing materials, I have discovered magnesia cements to be superior to all materials previously suggested for the same 75 purpose, namely cements composed of magnesium carbonate or oxide, combined with magnesium chloride. I have also found that the impurities found in commercial magnesite (which contains approximately 70 percent of magnesium salts and approximately 5 percent of water) will not interfere with the use of ordinary magnesite as this body material, thereby considerably reducing the cost of the stone. Furthermore, I have 80 found that by employing a suitable proportion of another salt of magnesium, namely magnesium sulphate (which is commercially available under the name of Epsom salts), I can retard the drying of the magnesia cement so as to increase the hardness 85 of the resulting stone to such a degree that the detached particles of copper will not imbed themselves into it.

90 In manufacturing a finish-grinding and polishing stone for use on copper printing plates, I have found the following proportions satisfactory: magnesite 40 ounces, crocus 48 ounces, jeweler's rouge 8 ounces, Epsom salt 8 ounces, magnesium chloride 100 16 ounces, water 3 pints.

The magnesite, crocus and rouge are first sifted separately through screens (desirably 300 mesh) and then thoroughly mixed while dry, while the magnesium chloride and the 105 Epsom salts are dissolved in the water to form a solution. The mixture of the sifted dry ingredients is then worked up with this solution to a mass of uniform consistency, which is forced through a screen (desirably 110 of about 50 mesh, for breaking up lumps and subdividing the plastic mass evenly)

into a bronze mold which has previously been waxed to prevent the mass from adhering to it. Left exposed to the air at ordinary temperatures, this plastic mass 5 hardens in from 24 to 30 hours to form the desired stone.

In the finished stone, the abrasive (crocus) and the polishing ingredient (rouge) form nearly one half of the entire weight, or 10 about double the proportion of the active ingredients in artificial stones heretofore proposed for the same purpose, so that my stone is unusually efficient in proportion to its weight and size. Moreover, the magnesia cement when thus diluted by the abrasive ingredient is in itself an abrasive of a degree of hardness suitable for having a grinding action on copper, thereby increasing the effectiveness of my stone. 15 20 In using such a stone for wet grinding, I have found that the surface wears evenly, and that the water and the grinding portions of the body material form the so-called "muck" in a desired consistency for carrying off the detached particles of copper. I have also found that any marks still left in the copper (if any) are so fine as to require only a quite small amount of hand polishing to remove them. More- 25 30 over, no poisonous materials are employed in the manufacture of my stone, so that I eliminate the danger heretofore encountered in making such stones with litharge as an ingredient of the body material.

35 However, I do not wish to be limited to the above mentioned proportions of the various ingredients or to the above recited procedure in the manufacture of my stones, since changes might obviously be made 40 without departing from the spirit of my invention and from the appended claims. Nor do I wish to be limited to the crocus as the abrasive or to rouge as the polishing ingredient when such an ingredient is also 45 employed, or to the use of the stones of my invention for grinding copper.

For example, the degree of fineness of the

grinding can be varied by sifting the crocus through a different size of mesh. The hardness of the body material can be modified 50 by varying the proportion of the retarder (such as Epsom salt) used with it, thereby correspondingly modifying the grinding action of this body material and also adapting this material to prevent the adhering of 55 detached particles harder than the copper of the usual printing plates.

I claim as my invention:

1. A stone for grinding and polishing copper, comprising a hardened and abrasive cement softer than copper and uniformly impregnated with a finely powdered abrasive and finely powdered rouge, the abrasive being harder than copper, the total weight of the abrasive and rouge being more than 65 forty per cent of the weight of the stone.

2. A grinding stone comprising the hardened product of an intimate mixture of a magnesia salt or salts, a finely divided abrasive and a finely divided polishing mate- 70 rial, with an aqueous solution of magnesium chloride mixed with a relatively small proportion of magnesium sulphate.

3. A grinding stone comprising a magnesia cement hardened under the influence 75 of a retarder and uniformly impregnated with a mixture of finely ground crocus and rouge, the proportion of the crocus to the rouge being about eight to one, and the total weight of the crocus and rouge being 80 more than forty percent of the weight of the stone.

4. A grinding stone comprising the product resulting from the hardening of the plastic mass produced by intermingling the 85 following ingredients in approximately the proportions recited, namely: 40 ounces magnesite, 48 ounces crocus, 8 ounces jeweler's rouge, 8 ounces Epsom salts, 16 ounces magnesium chloride and 3 pints 90 water.

Signed at Chicago, Illinois, March 16th, 1927.

ERNEST P. MARS.